

# UNITED STATES PATENT OFFICE.

JOHN A. KYLE, OF CHICAGO, ILLINOIS.

## MATERIAL FOR PROTECTING SHEETS, &c., IN TINNING.

No. 842,212.

Specification of Letters Patent.

Patented Jan. 29, 1907.

Application filed April 4, 1906. Serial No. 309,894.

*To all whom it may concern:*

Be it known that I, JOHN A. KYLE, a subject of the King of England, residing at Chicago, in the county of Cook and State of Illinois, have invented certain new and useful Improvements in Material for Protecting Sheets, &c., in Tinning, of which the following is a specification.

My invention consists in the production of a new material used in the manufacture of tin and terne sheets to be employed in covering the tin or lead bath, so as to prevent oxidation of the bath and of the coated surface of the sheet while the metal is solidifying, and the same is designed as an improvement upon or substitute for the material employed for the same purpose as described and claimed in my prior Letters Patent of the United States, No. 679,972, dated August 6, 1901.

The object of my present invention is to provide an improved material of the character described having such properties or constituencies that a plate may be produced which is practically free from blemish or fog, as well as free from black specks, which results are important and valuable in the tin-plate industry.

A further object of my invention is to provide a material of said character which shall retain its fluidity in continued use and shall minimize the tendency to become blackened.

I have discovered that a better product of tin-plate can be produced if, instead of using simply a fatty acid or acids and a petroleum product—such as, for instance, described and claimed in my patent aforesaid—I incorporate a small proportion of a glycerid of what is known chemically as the “non-drying” class—that is, a glycerid which is practically non-oxidizable by air at the temperature of the metal-coating bath and has the property

of remaining fluid even when maintained in contact with the air at a relatively high temperature, which is the case with my said material, inasmuch as the temperature of the tinning or metal-coating bath is about 600° Fahrenheit, more or less. The amount of the glycerid necessary in my improved compound or material to produce the desired results is relatively small, and I now consider that fifteen (15) per cent. is the maximum that need be used.

The glycerid which I prefer to employ is castor-oil obtained by pressure or any other means from what is known as the “castor-

bean;” but I do not wish to be understood as limiting myself to the use of this particular glycerid, so far as my broader claims are concerned, inasmuch as I may employ any glycerid, either of an animal or vegetable source, which practically cannot be oxidized or caused to solidify by the action of the air at the temperature of the metal-coating bath, which in practice is 600° Fahrenheit, more or less, in the case of tin, and 700° Fahrenheit, more or less, in the case of lead. In practice and referring to my preferred method of producing my said improved material or compound I mix with said glycerid a petroleum product of the same class as referred to in my Letters Patent aforesaid—that is, having a fire test of 400° to 725° Fahrenheit, more or less. According to the proportions which are preferred I take about one part of the glycerid to four parts of the petroleum product, although, as will be understood, these particular proportions may be varied somewhat. With this mixture of the glycerid and petroleum product I now incorporate as a component part of my material and also to insure a solution of the glycerid a fatty acid or fatty acids, which solidify at or above, say, 68° Fahrenheit and which are practically non-oxidizable by the air at the temperature of the metal-coating bath. This fatty acid or fatty acids may be either of an animal or a vegetable source and may be prepared in the manner set forth in my Letters Patent aforesaid. The proportions of fatty acid or fatty acids to the said mixture of glycerid and petroleum product or glycerids and petroleum product should be about one part of the former to three parts of the latter; but such proportions may be modified somewhat without departing from the spirit and scope of my invention.

In practice the completed compound is now heated up and maintained for some time at the melting-point of tin, which is about 450° Fahrenheit, and the same is then cooled and filtered to remove any vegetable or animal fiber or other extraneous matter which may have become coagulated or separated during said heating operation. The material or compound is now ready for use in the manner now well known in the art. This filtering of the material is desirable for removing such extraneous matters which, if not removed eventually carbonize and form objectionable black specks on the plate.

I claim—

1. A material for use in coating sheets with metal consisting of a fatty acid, a glycerid, and a solvent for such fatty acid and glycerid, said acid and glycerid being non-oxidizable at the temperature of the metal-coating bath; substantially as described.
2. A material for use in coating sheets with metal consisting of a fatty acid, a petroleum product, and a glycerid, said acid and glycerid being non-oxidizable at the temperature of the metal-coating bath; substantially as described.
3. A material for use in coating sheets with metal consisting of a fatty acid solidifying at a temperature of substantially 68° Fahrenheit, a petroleum product, and a glycerid non-oxi-

dizable at the temperature of the metal-coating bath; substantially as described.

4. A material for use in coating sheets with metal consisting of a fatty acid, castor-oil, and a solvent for such fatty acid and castor-oil, said acid being non-oxidizable at the temperature of the metal-coating bath; substantially as described.

5. A material for use in coating sheets with metal consisting of a fatty acid, castor-oil, and a petroleum product, said acid being non-oxidizable at the temperature of the metal-coating bath; substantially as described.

JOHN A. KYLE.

Witnesses:

S. E. HIBBEN,  
LOUIS B. ERWIN.